

# UNITED STATES PATENT OFFICE.

PAUL EMILE PLACET, OF PARIS, FRANCE.

## IMPROVEMENT IN PHOTO-GALVANOGRAPHY.

Specification forming part of Letters Patent No. 43,821, dated August 9, 1864.

*To all whom it may concern:*

Be it known that I, PAUL EMILE PLACET, of Paris, in the Empire of France, have invented certain new and useful Improvements in Engraving; and I hereby declare that the following is a full, clear, and exact description of the same.

My invention consists in new process for producing, without the aid of the engraver or of artistic "retouching" of photographic impressions, ornamental designs, engraved plates, &c., by means of divers manipulations or *modus operandi*, in the manner as follows: A plate is coated with a substance which light renders insoluble. After it is dry it is exposed, under a stereo or other like plate or surface carrying the design to be engraved, (cliché,) to the action of the light, and the portions not affected by the light are then dissolved. The insoluble parts appear upon the plate in relief, a cast of which being taken and reproduced by galvano-plastic process produce an engraved plate of the drawing, whose lines, however, are neither fine nor presenting the semi-tints possessed by the model. In the parts in which the semi-tints prevail the light does not render the coating insoluble throughout its whole thickness. The lines are therefore undermined by the dissolving agent, and are thus too frail to resist the washings attending the manipulations and are frequently carried off, together with the soluble matter underneath. This will evidently not take place if a suitable support be given to the insulated face and if the dissolving agent be caused to act upon the side opposite. In this way the subjectile will retain the semi-tints, and engraved plates may be produced therefrom from a cast by galvano-plastic process, which will have the fineness of the model. To carry this into effect I proceed as follows: I take an impression on a plate of glass of the "cliché" sought to be produced. On this impression or drawings I spread a coat of Judea bitumen or other like sensitive matter. I then expose to the light the glass side. When this is effected I plunge the plate in a mixture of naphtha and benzine. The parts rendered insoluble by the action of the light will constitute reliefs more or less pronounced, according to the length of time of exposure to light, the sensitiveness of the matter employed, and the nature of the cliché. Judea bitumen pro-

duces a very delicate engraving, but of little relief or depth. I therefore prefer to employ a mixture of gelatine with bichromate of potassa or ammonia. If on dissolving the soluble portion it is found that the reliefs are insufficient or too transparent, they may be increased by applying another coat of the sensitive matter, or by operating otherwise, in the same manner as at first.

This process is also applicable to the production of engraved plates, as described, from engravings or prints from engraved plates on paper. The paper should then be made transparent and impervious to the dissolving agents. Thus when bitumen is used as the sensitive matter with which the plate is coated the paper is first rendered impervious by dipping it in a solution of gelatine, gum, dextrine, or other like substance.

The operations must be varied according to circumstances. For producing engraved plates without directly operating on a proof or print the coating is applied to a thin plate of glass, gelatine, mica, horn, or other transparent body, and the plate is acted upon by the luminous rays on the side of the support. The coagulation thus proceeds from the face which is in contact with the support, and the design, after washing, remains a fixture on the supporting medium.

Another mode of proceeding is as follows: On a plate of glass two or more coats of collodion, then a coat of bichromated gelatine, are spread. After drying the same the borders of the gelatine are cut. It is then easily detachable, carrying with it the collodion, which forms body with it. The plate thus prepared is exposed to light under a cliché on the collodionized side, a plate of metal coated with some adhesive substance is applied to it, and the two are passed through a pair of rollers of a rolling-press. The sheet is then united with the plate while the gelatinized plate which is not impressioned is in the proper condition to be operated upon by the dissolving agents. A single coat of collodion does not suffice to secure easy detachment of the sheet; but instead of the collodion other substances having analogous properties may be used. After insulation, in order to give greater adherence of the collodion to the subjectile, it is preferred to spread a coat of varnish upon the collodion.

Another mode of proceeding is as follows: A thin but level-surfaced plate of metal is covered with the sensitive compound—say bichromated gelatine. After drying a coat of collodion is applied and the plate is exposed to the sun under a cliché. A fresh coat of collodion mixed with varnish, or a coat of varnish alone, is then applied, and finally a coating (sixteenth of an inch thick) of wax and resin is put on; or a metal disk is stuck on, as in the preceding case. After cooling, the thin metal plate is easily detached, leaving the sheet of gelatine to adhere to the subjectile with the insulated face above. Otherwise I proceed as in the preceding case. The first coat of collodion would penetrate the gelatine with less uniformity if applied after insulation, because the light renders the parts attacked less pervious. The coating of wax and resin has for its object to maintain the engraving upon a solid and even foundation by preventing the collodion to work, and thus to disfigure the design. The wax and resin may, however, be dispensed with by combining several coats of collodion and varnish, so as to neutralize the effects of contraction and expansion of the subjectile. The dissolving agent, acting upon the non-insulated side, commences by swelling the parts not impressioned and produces very beautiful and sharp reliefs. In many cases these reliefs may be utilized. A cast may be taken from them after the molding, before referred to, inasmuch as nothing prevents the action of the dissolving agent, in order to obtain a second engraving, which would be the inverse of the first. Thus one coat of sensitive matter may produce two engravings, one by the swelling of the parts non-impressioned, the other by dissolving the parts less soluble.

In lieu of the two substances before referred to—to wit, Judea bitumen and bichromated gelatine—many vegetable and animal matters may be used—such as resinous, gummy, albuminous, glutinous, and other like substances which are sensitive to light—either alone or when combined with other salts—such as salts of gold, silver, urane, chrome, iron, sulphurets,

iodurets, tartaric acid, oxalic acid, sal-ammonia, &c.

The operations are simplified by the employment of substances which, in the first place, are insoluble and become soluble under the action of light. There are many substances that possess this property. It is unnecessary, if not impossible, to enumerate them; but I may mention mixtures of gelatine, or gum, or albumen with a salt of iron, together with tartaric acid. If either of these mixtures be used, the salt of iron should be entered to its maximum. In the latter case the dissolving agent commences its action on the insulated face and corrodes very much in the same manner as the acid does in the etching process, but with this advantage, that the lines produced by the dissolving agent are more accurately defined and produce an intensity or shade corresponding to the cliché.

If in the composition of the sensitive coat certain vitrifiable substances are introduced as ingredients, and if these are caused to adhere to the reliefs after their formation, enamelled surfaces may be produced.

Upon the relief-surface printing or fat ink may be distributed, and the relief may be then dissolved, and the ink may be transferred on a stone or zinc, which may then be operated upon by the process of lithography.

Having thus described my invention, I claim—

The method of producing engraved surfaces by employment and application of substances which light renders insoluble to and upon the side of the subjectile which is directly exposed to the light, in combination with the dissolving operations, and the production of reliefs or plates engraved in intaglio by molding or galvano-plasty, substantially as herein described.

In testimony whereof I have signed my name to this specification before two subscribing witnesses.

P. EM. PLACET.

Witnesses:

E. JAUME,  
E. SHERMAN GOULD.